

Dec. 31, 1929.

E. R. WEHR ET AL

1,741,388

METAL COATING METAL SHEETS

Filed Sept. 13, 1926



INVENTOR  
Earl R. Wehr - Carl O. Mahle  
BY  
Albert Allen  
ATTORNEYS

## UNITED STATES PATENT OFFICE

EARL R. WEHR AND CARL C. MAHLIE, OF MIDDLETOWN, OHIO, ASSIGNEES TO THE AMERICAN ROLLING MILL COMPANY, OF MIDDLETOWN, OHIO, A CORPORATION OF OHIO

## METAL COATING METAL SHEETS

Application filed September 13, 1926. Serial No. 135,275.

Our invention relates specifically to the formation of a coating on steel and iron sheets which consists on the surface at least of an alloy of zinc and aluminum, but inasmuch as certain of the steps would also be applicable to the formation of alloy coatings of different metals on metallic bodies capable of being fed through a bath, the invention has more general aspects as will subsequently appear.

In the coating of sheet metal by the method of feeding it through molten metal baths, and particularly with iron and steel, when subjected to surface treatments with metals which coat the iron, the problem of securing a proper coating is rendered difficult because of the large area which must be covered and because of the distinctness with which any defect appears on the large flat area.

The process is also rendered difficult due to the fact that the ordinary fluxes can not be used on a bath consisting of zinc and aluminum because of the formation of aluminum chloride ( $AlCl_3$ ) which volatilizes readily at the temperature of the bath.

We employ as the main portion of the bath, molten lead, with a flux box at the entrance end, and an exit box at the exit end, in which exit box is maintained a floating molten body of zinc aluminum alloy.

Our process has considerable by way of advantage, due to the fact that we preferably employ commercially pure zinc in forming the zinc-aluminum alloy. Pure zinc will dissolve to a small extent in the lead bath, but the lead will be insufficiently changed to enable it to take up the aluminum. In machine processes, with which we are dealing, the continued passage of material through the bath, with continued additions of the floating alloy in the exit compartment on the lead bath will soon deteriorate the bath, if this is possible. But lead will take up only so much zinc, and this will not enable it to dissolve the aluminum to any appreciable extent, with the result that high aluminum alloys can be kept at the exit end of the machine, floating on the lead, without aluminum getting into the lead and defiling

it sufficiently to render the fluxing problem difficult.

With alloys high in aluminum as a coating, we are fairly closely confined to the use of commercially pure zinc, as the main body of the floating coating material. 55

By our process we can produce a continuous succession of iron or steel sheets coated with an alloy of zinc and aluminum, quite high in aluminum, say up to twenty percent aluminum. Above twenty percent aluminum, the melting point of the alloy gets higher than the melting point of pure zinc, which introduces another problem that we avoid by keeping below twenty percent aluminum. 60

Normally it will be of little value to use three percent or less of aluminum, as the product produced does not vary sufficiently to give the very decided novel product that is produced by us. For example, a coating 70 containing commercially pure zinc, and eight percent of aluminum by weight to the zinc, has proven to be a radical departure and improvement over past products, and producible by our process without excessive expense, with avoidance of any hand dipping, or fluxing previous to introduction into the machine. 75

Normally it will be of little value to use three percent or less of aluminum, as the product produced does not vary sufficiently to give the very decided novel product that is produced by us. For example, a coating 70 containing commercially pure zinc, and eight percent of aluminum by weight to the zinc, has proven to be a radical departure and improvement over past products, and producible by our process without excessive expense, with avoidance of any hand dipping, or fluxing previous to introduction into the machine. 75

We accomplish our objects by that certain process to be hereinafter more specifically pointed out and claimed. 80

In the drawing, the figure is a diagram of equipment found by us to be satisfactory with our process.

We have shown coating equipment having 85 a pot 1, with guides 2, exit rolls 4, and flux box 5. The exit rolls have located alongside of them stirring or skimming rolls 6. A partition 7 extends down into the pot dividing the upper portion of the bath. The alloys we use deteriorate the pot rapidly, so that care must be taken in the metals used in avoiding a product soluble in the alloy. 90

In this process, pure lead is melted in the pot to the desired level. Zinc-aluminum alloy is melted on top of the lead at the exit end, and a small amount of pure zinc is melted in the flux box on top of the lead. Any of the usual galvanizing fluxes can be used on the zinc, such as sal-ammoniac. The 100

use of pure zinc at these points is desirable as against impure zinc spelters, where the finish of the sheet is to be of the highest value and free from the typical spangle, and to avoid contamination of the zinc aluminum alloy at the exit end of the mechanism, and also for the reasons heretofore noted.

5 The level of the lead at the exit end is indicated at 8 upon which is the zinc-aluminum alloy 9. The level of the lead in the 10 flux box is indicated at 10 and the zinc in the flux box at 11.

15 The cleaned metal sheet is passed through the flux 12 into the zinc where it becomes zinc coated and then down through the lead, which partially replaces the zinc coating, and up through the zinc-aluminum alloy, which replaces the lead, the final product being coated with zinc-aluminum alloy.

20 The advantage of using a molten zinc on which the flux is supported lies in the fact that where the metal to be passed down through a flux supported on the lead, the flux often adheres in spots which are subsequently 25 coated over.

30 The percentage of aluminum in the zinc-aluminum alloy is maintained at any desired percentage. In one of our practices, we keep the alloy at around six per-cent aluminum, and in another we use eight per-cent.

35 We do not wish, however, to be excluded from covering the use of a flux directly on the lead even though the product is not so readily produced in uniform excellence, nor do we 40 wish to be limited to pure zinc alone in some phases of our process. By reference to alloys of zinc and aluminum in the claims that follow, we do not wish to exclude the presence of small quantities of other metals, so long as the aluminum is the important alloying element with the zinc.

Having thus described our invention, what we claim as new and desire to secure by Letters Patent, is:—

45 1. A process of coating metal sheets which consists of passing them through a flux into a molten body of zinc floating on a molten metallic bath of a heavier metal, down through said molten metallic bath of a heavier metal, 50 and up through a molten metallic body containing zinc and alloying material and floating on the molten bath of a heavier metal said heavier metal being such as will not substantially absorb said zinc alloy.

55 2. A process of coating metal sheets which consists of passing them through a flux and into a molten body of pure zinc floating on molten lead, and down into the molten lead bath and through the lead bath up through a 60 molten metal body containing zinc and aluminum floating on the lead.

65 3. A process of coating ferreous sheets which consists of passing them through a flux, into a molten body of pure zinc floating on a molten bath of lead, and through the molten

bath of lead and up through a molten body of zinc-aluminum alloy floating on the molten lead bath, the zinc-aluminum alloy being kept from access to the flux.

4. A process of coating metal bodies having a plane surface which comprises passing them through a flux, through a bath of molten lead, and out through a molten alloy floating on the surface of the lead, in a continuous manner, said alloy composed of commercially pure zinc and aluminum. 70

5. A process of coating metal bodies having a plane surface which comprises passing them through a flux, through a bath of molten lead, and out through a molten alloy floating on the surface of the lead, in a continuous manner, said alloy composed of commercially pure zinc and aluminum, said aluminum being present in quantities less than twenty percent by weight of the zinc, and more than five per 75 cent. 80

6. A process of coating metal bodies having a plane surface which comprises passing them through a flux, through a bath of molten lead, and out through a molten alloy floating on the surface of the lead, in a continuous manner, said alloy composed of commercially pure zinc and aluminum, said aluminum being present in quantities less than twenty percent by weight of the zinc, and over three percent 85 by weight of the zinc. 90

EARL R. WEHR.  
CARL C. MAHLIE.

100

105

110

115

120

125

130